

1

3,785,939

**TIN/LEAD PLATING BATH AND METHOD**  
Grace F. Hsu, Vernon, Conn., assignor to Conversion  
Chemical Corporation, Rockville, Conn.  
No Drawing. Filed Oct. 22, 1970, Ser. No. 83,229  
Int. Cl. C23b 5/38, 5/40, 5/46

U.S. CL. 204—43 S

23 Claims

## ABSTRACT OF THE DISCLOSURE

A plating bath for electrodeposition of tin/lead alloys contains stannous ion, lead ion, a fluoroborate, fluosilicate or sulfamate radical and, as a brightener system, a non-ionic polyoxyalkylated surfactant, a lower aliphatic aldehyde, an aliphatic or aromatic amine and an aromatic aldehyde, the pH of the bath being less than about 3.0.

## BACKGROUND OF THE INVENTION

Electrodeposited tin/lead alloys of different compositions are valuable in a number of applications including the provision of bearing contact surfaces (for which a 7/93 tin/lead alloy is typically used) and the provision of surfaces for soldering such as on printed circuit boards and the like (for which alloys of 60/40 tin/lead are desired). Although a number of formulations have been suggested for use in producing solder plate, it is believed that a significant need remains for a bath this is capable of producing a high quality tin/lead deposit having a composition at or near the eutectic value for the alloy (about 63/37), as it optimum for soldering purposes. Moreover, effective compositions for producing bright or semi-bright alloy electrodeposits have not been available commercially, and there is a widespread demand for a practical way of producing such deposits on articles of various types for both technical and also aesthetic reasons. It is also desirable that such deposits retain their solderability over extended periods of time, and either be resistant to discoloration or be adapted to facile treatment to prevent such discoloration.

Accordingly, it is an object of the present invention to provide a novel electroplating bath that is capable of producing relatively bright deposits of tin/lead alloy.

It is also an object of the invention to provide such a bath that is capable of producing the metal deposits with good current efficiency, that is operable over a broad range of current densities and that exhibits good covering power.

Another object is to provide workpieces having an optimum tin/lead alloy electrodeposit for soldering, where the composition is at or near the eutectic point for tin/lead alloys and is at least relatively bright.

Still another object is to provide an electroplating method for the production of high quality tin/lead alloy deposits, which method is efficient and effective, is conducted under convenient conditions, and is capable of producing bright solderplate deposits.

## SUMMARY OF THE DISCLOSURE

It has now been found that the foregoing and related objects can be readily attained in an aqueous acid plating bath for the electrodeposition of tin/lead alloys comprising about 5.0 to 80.0, and preferably about 45.0 to 65.0, grams per liter of stannous ion; about 85.0 to 10.0, and preferably about 35.0 to 15.0, grams per liter of lead ion; and at least about 100.0, and preferably at least about 150.0, grams per liter of a radical selected from the group consisting of fluoroborate, fluosilicate, and sulfamate. The bath also includes, as a brightener system, at least about 5.0 grams per liter of a nonionic polyoxyalkylated surfactant, at least about 4.0 grams per liter of a lower aliphatic aldehyde containing 1 to 4 carbon atoms, at

least about 2.0 grams per liter of an amine, and at least about 0.25 gram per liter of an aromatic aldehyde; the bath has a pH of less than about 3.0. Preferably, the amount of the components of the brighteners system are 5 10.0 to 30.0, 5.0 to 15.0, and 0.4 to 1.5, grams per liter, respectively, and the pH of the bath is most desirably below about 1.0.

In the preferred embodiments, the brightener system of the bath includes at least about 2.0 grams per liter of an aromatic amine, and the aromatic aldehyde is ring-halogenated. Most desirably, the aromatic aldehyde is either 10 2,4-dichlorobenzaldehyde or orthochlorobenzaldehyde, and it is used in an amount of about 0.5 to 2.0 grams per liter. When the bath utilizes the fluoroborate radical, as 15 is preferred, it desirably also contains at least about 50.0 grams per liter of free fluoroboric acid and at least about 10.0, grams per liter of free boric acid. The aromatic amine employed is desirably selected from the group consisting of toluidines and aniline, and is preferably 20 either ortho- or meta-toluidine included in an amount of about 3.0, to 12.0 grams per liter. The lower aliphatic aldehyde that is used is preferably formaldehyde, and it is preferably present in an amount of about 5.0 to 15.0 grams per liter. If desired, the bath may additionally 25 include about 0.5 to 7.5 grams per liter of an additive selected from the class consisting of peptone, resorcinol, glue, gelatine, betanaphthol, polyvinyl alcohol, cresylic acid, and mixtures thereof. Advantageously, it includes about 0.5 to 2.0, grams per liter of cresylic acid.

Certain objects of the invention are also readily attained in a method of electroplating tin/lead alloys wherein a bath having a composition as hereinbefore described is first prepared. The bath is maintained at a temperature of at least about 50° Fahrenheit, and a workpiece having 35 a metallic surface and at least one anode to provide the necessary tin and lead anodic supply are immersed therein. Thereafter, a voltage is applied across the anode and the workpiece to deposit tin and lead on the metallic surface, and the voltage applied provides a current density at the workpiece of about 10 to 200 amperes per square foot.

Preferably, there is utilized an alloy anode having a composition of approximately 60.0 percent by weight of tin and 40.0 percent by weight of lead. Alternatively, 45 at least two anodes may be immersed in the bath, one of which consists essentially of tin and the other of which consists essentially of lead, with the method including the step of apportioning the current between the anodes so as to deposit tin and lead upon the workpiece in the desired proportions.

## DETAILED DESCRIPTION OF THE PREFERRED EMBODIMENTS

The bath electrolyte is preferably provided by the fluoroborate, fluosilicate, or sulfamate salts of tin and lead, although other salts may be used to furnish all or a portion of the tin and lead ions, and the desired radical may be provided by a suitable acid, such as fluoroboric. It should be appreciated that the foregoing terms are used generically herein, and may encompass the more complex salts such as the phenolsulfamate compounds. In any event, the amount of stannous ion provided must be in the range of about 5.0 to 80.0 grams per liter and the amount of lead ion employed therewith must range from about 85.0 to 10.0 grams per liter. Preferably, the amount of stannous ion will exceed the lead ion and will be in the range of about 45.0 to 65.0 grams per liter, with the amount of lead ranging from about 35.0 to 15.0 grams per liter. A most desirable feature of the invention is that it enables the formation of electrodeposits of solder having a composition at or near the eutectic point for tin/lead alloys, and the most desirable range of the ions in the bath therefor is 55 60 65 70

about 53.0 to 57.0 grams of stannous ion per liter and about 27.0 to 23.0 grams of lead ion per liter.

The fluoborate baths are preferred and, to be satisfactory, must contain at least about 100.0 grams per liter of the fluoborate radical; preferably the amount of the radical will be not less than about 150.0 grams per liter. Such a bath should contain at least about 50.0 grams per liter of fluoboric acid and at least about 10.0 grams per liter of boric acid.

A typical "make-up" formula (brightening system and additives omitted) for a liter bath, that has performed well, is as follows (percentages expressed being by weight):

|                                  |             |      |
|----------------------------------|-------------|------|
| Stannous fluoborate concentrate: | grams       | 272  |
| 49.6% stannous fluoborate        |             |      |
| 1.8% fluoboric acid              |             |      |
| 2.0% boric acid                  |             |      |
| Lead fluoborate concentrate:     | do          | 92.8 |
| 51% lead fluoborate              |             |      |
| 0.6% fluoboric acid              |             |      |
| 1.9% boric acid                  |             |      |
| Fluoboric acid (49%)             | milliliters | 142  |
| Boric acid                       | grams       | 18.3 |

The foregoing formulation provides about 60.0 grams per liter of total tin (about 55.0 grams per liter of stannous ion and about 5.0 grams per liter of stannic ion) about 25.0 grams per liter of lead ion, about 100.0 grams per liter of fluoboric acid (absolute), and about 25.0 grams per liter of boric acid.

In accordance with the concept of the present invention, the foregoing type of make-up formulation (be it of the fluoboric, fluosilicate, or sulfamate variety) must also contain a brightener system comprised of at least about 5.0 grams per liter of nonionic polyoxyalkylated surfactant, at least about 4.0 grams per liter of a lower aliphatic aldehyde, and at least about 0.25 gram per liter of an aromatic aldehyde. Preferably, the amounts of the foregoing components will be about 10.0 to 30.0, 5.0 to 15.0, and 0.4 to 1.5, grams per liter, respectively.

As regards the specific composition of the nonionic surfactant, virtually any surface active polyoxyalkylated compound that is soluble in the bath may be employed, and a wide variety of such materials are commercially available under a number of different trademarks. However, the polyethoxylated fatty acid monoalkanolamides and related amines, and the polyethoxylated alkylphenols have performed particularly effectively. Exemplary of the polyethoxylated fatty acid monoethanolamides that may be used to advantage are the cocoanut fatty acid and lauric acid derivatives sold by Stepan Chemical Company of Northfield, Ill. under the trademarks Amidox C-5 and Amidox L-5, respectively. Exemplary of the polyethoxylated alkylphenol surfactants that may advantageously be used is the ethoxylated nonylphenol derivative sold by Onyx Chemical Company of Jersey City, N.J., under the trademark Neutronyx 675. Substitution of similar materials is contemplated and encompassed within the scope of the invention, and specific alternative surfactants will be apparent to those skilled in the art, in view of the foregoing disclosure.

With regard to the specific lower aliphatic aldehyde constituent, it should contain 1 to 4 carbon atoms and, although acetaldehyde, butyraldehyde and propionaldehyde may be employed, formaldehyde is preferred.

The specific composition of the aromatic aldehyde may also vary considerably within the scope of the invention. Although it may be feasible to use unsubstituted and alkyl substituted benzene nuclei, and multicarbon chain aldehyde groups, including benzaldehyde, tolualdehyde, cinnamaldehyde, etc., the ring-halogenated benzaldehydes are preferred, and particularly desirable results have been found to result from the use of either ortho-chlorobenzaldehyde or 2,4-dichlorobenzaldehyde. In any event, it is essential to the proper operation of the baths described

herein that at least one lower aliphatic aldehyde and at least one aromatic aldehyde be employed therein; combinations of two or more of each species of aldehyde may also be employed in some instances.

In addition to the foregoing components, and in accordance with the preferred embodiments, various additives and adjuvants may be included in the plating formulation. A particularly desirable adjuvant is a compound furnishing an amine group, including both aliphatic and aromatic amines. Although aliphatic amines such as butylamine and the like have been effective, particularly outstanding improvements have been noted to result from the inclusion of aromatic amines, and especially from the use of ortho-toluidine, meta-toluidine and aniline. When employed, the amine should be used in an amount of no less than about 2.0 grams per liter; preferably the amount will be between 3.0 and 12.0 grams per liter, and most desirably about 4.0 grams per liter thereof will be used.

Among the other additives which may be included to modify the operation of the present bath are auxiliary surfactants, secondary brighteners, and other materials, such as the polyvinyl alcohols, peptone, resorcinol, glue, gelatine, beta-naphthol, etc., which should usually be added in amounts of about 0.5 to 7.5 grams per liter. It has been found that use of about 0.5 to 5.0 grams per liter of cresylic acid is a particularly desirable expedient since it improves the smoothness of the deposits obtained to a considerable degree. Although little or no tendency for metal sludge or precipitate formation has been noted in baths properly operated in accordance with the invention, in some instance it may be desirable to incorporate a chelating agent such as citric acid, malic acid, or the aminopolyacetic acids (e.g. ethylenediamine tetraacetic acid, ethylenetriamine pentaacetic acid, nitrilotriacetic acid). Such chelating agents, when employed, are generally included in an amount of about 5.0 to 20.0 grams per liter.

Since some of the suitable brighteners and other components which may desirably be included in the bath exhibit relatively low solubility therein, it may be necessary or desirable to employ a solvent solution thereof to facilitate formulation of the bath. Among the various solvents that may be employed, depending upon the particular component involved, are the low molecular weight alcohols (methanol, ethanol, and propanol) and the low molecular weight glycol ethers (ethylene glycol monomethyl ether, etc.). Generally, the component will be added as a 0.1 to 5.0 and preferably as a 0.5 to 2.0 percent by weight solution so as to obtain a stable solvent solution which may be readily dispersed in the acid bath.

A typical brightener system found to produce outstanding bright solder plate deposits, in combination with the typical "make-up" formulation hereinbefore described, has the following composition, on a liter basis:

|                                                                     | Milliliters |
|---------------------------------------------------------------------|-------------|
| Polyethoxylated fatty acid monoethanolamide surfactant (Amidox C-5) | 15          |
| Ortho-toluidine                                                     | 6           |
| Formaldehyde (37 weight percent in water)                           | 30          |
| 2,4-dichlorobenzaldehyde (10 weight percent in methanol)            | 6           |

As has been indicated previously, the baths of the present invention are operable over a fairly wide range of cathode current density, depending upon other factors such as temperature, agitation, etc. More specifically, the operable range is about 10.0 to 200.0 amperes per square foot (a.s.f.) and preferably about 20.0 to 120.0 a.s.f., with a narrower range of 25.0 to 35.0 a.s.f. being most desirable for the production of deposits having a substantially eutectic composition. The plating efficiency is generally quite high and will range up to about 95 percent under optimum conditions, based upon the theoretical rate of deposition, and bright deposits of excellent quality can best be produced at a bath efficiency in

excess 70 percent. The applied voltage should be about 0.2 to 5.0 volts and preferably 0.5 to 4.0 volts.

The baths should be operated at a temperature of at least about 50° Fahrenheit, and preferably from about 60 to 90° Fahrenheit. Operation below about 50° Fahrenheit tends to be inefficient and to produce undesirable deposits, whereas temperatures higher than about 90° Fahrenheit tend to cause oxidation of the tin ion to the stannic state and to produce dull, rough and generally unacceptable deposits; furthermore, the bath is consumed at an excessive rate at temperatures that are unduly high.

Any metallic substrate or metal-surfaced article which can be plated with tin using prior art baths may be coated in accordance with the present invention. For example, good deposits may be produced upon articles of copper, nickel, iron, steel, etc. The best results are obtainable with these baths if relatively pure anodes of the metals are employed, and either tin/lead alloy anodes or separate tin anodes and lead anodes may be used. It should be noted that the composition of the anode has a significant effect upon the composition of the deposit, and that it is generally desirable to employ an anode having a proportion of metal approximating that desired in the plated alloy. The composition of the deposit may also be controlled by use of separate anodes of tin and lead, to which the current may be proportioned appropriately.

Some agitation is desirable to obtain high quality, uniform deposits and to avoid development of sludge or film, and plating at high current densities and temperatures may be improved by more intense agitation. However, excessively high rates of agitation are undesirable because they can cause excessive consumption of the bath and impose limitations upon the current densities at which brightness is achieved. Not only is agitation of the bath itself desirable but agitation of the cathode may be beneficial in obtaining a uniform plate and enabling extension of the range of satisfactory current density.

The process is adapted to still plating and barrel plating apparatus with equal efficacy, and may be used for strip, wire and connector strip. Use of the bath and process is particularly significant with respect to connector strip, printed circuit boards, and the like because of the excellent solderability of the plate produced. Filtration of the bath is not essential but will normally be beneficial when contamination of the bath is encountered due to air-borne impurities and carryover from other finishing operations; preferably, it will be effected on a continuous basis. Various filtering media may be utilized including fabrics, such as of polypropylene, and other conventional filtering materials.

The depletion of the various components of the bath is best corrected by analysis for the several components on a periodic basis which can be established for a given facility. To determine the amounts of stannous salt required, an iodine titration technique may be used; the lead content may be checked by precipitation with dilute sulfuric acid. The amount of the surfactant and other components may be best evaluated by testing a sample of the bath in a suitable test cell, and a suitable schedule may be established for a given facility and workpiece.

Illustrative of the efficacy of the present invention are the following specific examples, wherein all percentages are on a weight basis.

#### Example 1

An aqueous plating bath was prepared by admixing, with water, sufficient quantities of stannous and lead fluoborate concentrates (as set forth in the typical "make-up" formula hereinbefore recited) fluoboric acid, and boric acid, to provide 55.0 grams per liter of stannous tin (as metal), 100.0 grams per liter of fluoboric acid about 25.0 grams per liter of lead ion (as metal) and 25.0 grams per liter of boric acid. The bath also contained a brightener system consisting of about 15.0 milliliters per liter of an ethoxylated coconut fatty acid monoethanol-

amide containing 5 moles of ethylene oxide per mole of amide (sold by Stepan Chemical Company of Northfield, Ill. under the trademark Amidox C-5), about 6.0 milliliters per liter of ortho-toluidine, about 30.0 milliliters per liter of 37.0 percent formaldehyde, and about 6.0 milliliters per liter of a 10.0 percent methanol solution of 2,4-dichlorobenzaldehyde. About 7.5 milliliters per liter of a 10.0 percent methanol solution of cresylic acid was also included in the bath to improve the smoothness of the deposit, and the pH of the bath was less than 1.0.

Plating was effected in a Hull cell at room temperature, using as the anode an alloy of 60/40 tin/lead. The bright plating current density range was found to extend from about 10 to more than 120 amperes per square foot. Even below 10 a.s.f. the deposits were of good quality, albeit with a slightly milky appearance.

#### Example 2

In a series of barrel plating runs, the same formulation as was used in Example 1 is employed, the temperature and current density being varied to demonstrate the characteristics of the bath. As a result, it is found that the optimum temperature of operation is about 70°-85° Fahrenheit; higher temperatures are found to be less desirable since oxidation of tin to the stannic state is more pronounced and since operation is required within a higher current density range for bright deposits. At current densities of less than about 75 a.s.f., metal efficiency is found to be considerably higher than about 90 percent; at a current density of about 30 a.s.f. a nearly eutectic alloy, containing about 64 percent of tin, is produced. Mild agitation during plating is found to result in deposits of excellent appearance, the covering power is outstanding, and the throwing power of the bath appears to be very good, particularly for an acidic system.

Thus, it can be seen that the present invention provides a novel electroplating bath that is capable of producing relatively bright deposits of tin/lead alloy. The bath produces such deposits with good current efficiency and good covering power, and it is operable over a broad range of current densities. The invention provides workpieces having at least relatively bright tin/lead alloy electrodeposits in which the composition is at or near the eutectic point for such alloys, as is optimum for soldering, and the method provided is efficient and effective, may be conducted under convenient conditions, and is capable of producing high quality deposits, as previously described.

Having thus described the invention, I claim:

1. An aqueous acid plating bath for electro-deposition of tin/lead alloys comprising about 5.0 to 80.0 grams per liter of stannous ion; about 85.0 to 10.0 grams per liter of lead ion; at least about 100.0 grams per liter of a radical selected from the group consisting of fluoborate, fluorosilicate and sulfamate; and, as a brightener system, at least about 5.0 grams per liter of a nonionic polyoxyalkylated surfactant, at least about 4.0 grams per liter of a lower aliphatic aldehyde containing 1 to 4 carbon atoms, at least about 0.25 gram per liter of said bath of an aromatic aldehyde and at least about 2.0 grams per liter of said bath an amine, said bath having a pH of less than about 3.0.

2. The bath of claim 1 containing about 45.0 to 65.0 grams per liter of stannous ion and about 35.0 to 15.0 grams per liter of lead ion.

3. The bath of claim 2 wherein said radical is fluoborate and said bath contains at least about 150.0 grams per liter thereof, wherein said bath contains at least about 50.0 grams per liter of free fluoboric acid and at least about 10.0 grams per liter of free boric acid, wherein said lower aliphatic aldehyde is provided by about 5.0 to 15.0 grams per liter of formaldehyde, and wherein said pH is less than about 1.0.

4. The bath of claim 3 wherein said amine is furnished by about 3.0 to 12.0 grams per liter of an aromatic amine selected from the class consisting of ortho- and meta-

toluidines, wherein said surfactant is selected from the class consisting of ethoxylated fatty acid monoalkanolamides and ethoxylated alkylphenols and is present in an amount of about 10.0 to 30.0 grams per liter, and wherein said aromatic aldehyde is selected from the group consisting of 2,4-dichlorobenzaldehyde and ortho-chlorobenzaldehyde and is present in an amount of about 0.4 to 1.5 grams per liter.

5. The bath of claim 4 additionally including about 0.5 to 2.0 grams per liter of cresylic acid.

6. The bath of claim 1 wherein said aromatic aldehyde is a ring-halogenated aldehyde and wherein said amine is an aromatic amine.

7. The bath of claim 6 wherein said aromatic amine is selected from the group consisting of toluidines and aniline, and wherein said lower aliphatic aldehyde is formaldehyde.

8. The bath of claim 6 wherein said aromatic aldehyde is ring-halogenated.

9. The bath of claim 1 wherein said radical is fluoborate and said bath contains at least about 150.0 grams per liter thereof, wherein said bath contains at least about 50.0 grams per liter of free fluoboric acid and at least about 10.0 grams per liter of free boric acid, and wherein said pH is less than about 1.0.

10. The bath of claim 1 additionally including about 0.5 to 7.5 grams per liter of an additive selected from the class consisting of peptone, resorcinol, glue, gelatine, betanaphthol, polyvinyl alcohol, cresylic acid, and mixtures thereof.

11. The bath of claim 1 wherein said aromatic aldehyde is ring-halogenated.

12. In a method of electroplating tin/lead alloys, the steps comprising:

(a) preparing an aqueous acid plating bath comprising about 5.0-80.0 grams per liter of stannous ion, about 85.0-10.0 grams per liter of lead ion, at least about 100 grams per liter of a radical selected from the group consisting of fluoborate, fluosilicate and sulfamate and, as a brightener system, at least about 5.0 grams per liter of a nonionic polyoxyalkylated surfactant, at least about 4.0 grams per liter of a lower aliphatic aldehyde containing 1 to 4 carbon atoms, at least about 0.25 grams per liter of said bath of an aromatic aldehyde and at least about 2.0 grams per liter of said bath of an amine, said bath having a pH of less than about 3.0.

(b) maintaining said bath at a temperature of at least about 50° Fahrenheit;

(c) immersing a workpiece having a metallic surface and at least one anode providing tin and lead in said bath; and

(d) applying a voltage across said anode and workpiece to deposit tin and lead on said metallic surface, said voltage providing a current density of about 10 to 200 amperes per square foot at the workpiece.

13. The method of claim 12 wherein said anode contains approximately 60.0 percent by weight of tin and 40.0 percent by weight of lead.

14. The method of claim 13 wherein said voltage provides a current density of about 25 to 35 amperes per square foot at the workpiece to produce a tin/lead alloy thereon having a composition of about 62.0 to 64.0 percent by weight of tin, and conversely, about 38.0 to 36.0 percent by weight of lead.

15. The method of claim 12 wherein said amine is an aromatic amine selected from the group consisting of toluidines and aniline, wherein said lower aliphatic aldehyde is formaldehyde, and wherein said radical is fluoborate and wherein said pH is less than about 1.0.

16. The method of claim 15 wherein said aromatic amine is selected from the group consisting of ortho- and meta-toluidines, wherein said surfactant is selected from the class consisting of ethoxylated fatty acid monoalkanolamides and ethoxylated alkylphenols and is present in an amount of about 10.0 to 30.0 grams per liter, and wherein

said aromatic aldehyde is selected from the group consisting of 2,4-dichlorobenzaldehyde and ortho-chlorobenzaldehyde and is present in an amount of about 0.4 to 1.5 grams per liter.

17. The method of claim 12 wherein at least two anodes are immersed in said bath, one of said anodes consisting essentially of tin and the other of said anodes consisting essentially of lead, and wherein said method includes the step of apportioning the current between said anodes so as to deposit tin and lead in desired proportions upon the workpiece.

18. The method of claim 12 wherein said applied voltage provides a current density of about 20 to 120 amperes per square foot at the workpiece.

19. An aqueous acid bath for electrodeposition of tin/lead alloys comprising about 5.0 to 80.0 grams per liter of stannous ion; about 85.0 to 10.0 grams per liter of lead ion; at least about 100.0 grams per liter of a radical selected from the group consisting of fluoborate, fluosilicate and sulfamate; and, as a brightener system, at least about 5.0 grams per liter of a surfactant selected from the class consisting of ethoxylated fatty acid monoalkanolamides and ethoxylated alkylphenols, at least about 4.0 grams per liter of formaldehyde, at least about 2.0 grams per liter of an aromatic amine selected from the group consisting of toluidines and aniline, and at least about 0.25 gram per liter of a ring-halogenated aromatic aldehyde, said bath having a pH of less than about 3.0.

20. The bath of claim 19 wherein said radical is fluoborate and said bath contains at least about 150.0 grams per liter thereof, wherein said bath contains at least about 50.0 grams per liter of free fluoboric acid and at least about 10.0 grams per liter of free boric acid, wherein said aromatic amine is selected from the group consisting of ortho- and meta-toluidines, wherein said aromatic aldehyde is selected from the group consisting of 2,4-dichlorobenzaldehyde and ortho-chlorobenzaldehyde, and wherein said bath has a pH less than about 1.0.

21. The bath of claim 19 containing about 45.0 to 65.0 grams per liter of stannous ion, about 35.0 to 15.0 grams per liter of lead ion, about 5.0 to 15.0 grams per liter of formaldehyde, about 3.0 to 12.0 grams per liter of said aromatic amine, about 10.0 to 30.0 grams per liter of said surfactant, and about 0.4 to 1.5 grams per liter of said aromatic aldehyde.

22. In a method of electroplating tin/lead alloys, the steps comprising:

(a) preparing an aqueous acid bath comprising about 5.0 to 80.0 grams per liter of stannous ion; about 85.0 to 10.0 grams per liter of lead ion; at least about 100.0 grams per liter of a radical selected from the group consisting of fluoborate, fluosilicate and sulfamate; and, as a brightener system, at least about 5.0 grams per liter of a surfactant selected from the class consisting of ethoxylated fatty acid monoalkanolamides and ethoxylated alkylphenols, at least about 4.0 grams per liter of formaldehyde, at least about 2.0 grams per liter of an aromatic amine selected from the group consisting of toluidines and aniline, and at least about 0.25 grams per liter of a ring-halogenated aromatic aldehyde, said bath having a pH of less than about 3.0.

(b) maintaining said bath at a temperature of at least about 50° Fahrenheit;

(c) immersing a workpiece having a metallic surface and at least one anode providing tin and lead in said bath; and

(d) applying a voltage across said anode and workpiece to deposit tin and lead on said metallic surface, said voltage providing a current density of about 10 to 200 amperes per square foot at the workpiece.

23. The method of claim 22 wherein said radical is fluoborate and said bath contains at least about 150.0 grams per liter thereof, wherein said bath contains at least about 50.0 grams per liter of free fluoboric acid and at least about 10.0 grams per liter of free boric acid,

wherein said aromatic amine is selected from the group consisting of ortho- and meta-toluidines, wherein said aromatic aldehyde is selected from the group consisting of 2,4-dichlorobenzaldehyde and ortho-chlorobenzaldehyde, and wherein said bath has a pH less than about 1.0.

2,489,523 11/1949 Clifton ----- 204-43  
2,633,450 3/1953 Andrews ----- 204-54 R

## FOREIGN PATENTS

5 652,405 12/1964 Belgium ----- 204-54 R  
1,151,460 5/1969 Great Britain ----- 204-43

## OTHER REFERENCES

Abner Brenner: "Electrodeposition of Alloys," vol. II,  
pp. 11 and 12, (1963).

GERALD L. KAPLAN, Primary Examiner

## References Cited

## UNITED STATES PATENTS

|           |         |                     |           |
|-----------|---------|---------------------|-----------|
| 2,598,486 | 5/1952  | Andrews -----       | 204-54 R  |
| 2,460,252 | 1/1949  | DuRose et al. ----- | 204-43 10 |
| 3,471,379 | 10/1969 | Schoot et al. ----- | 204-54 R  |